

May 8, 1928.

E. H. O'NEIL

1,669,016

DEODORANT AND METHOD OF MAKING SAME

Filed Nov. 27, 1923

*Fig. 1.*



*Fig. 2.*



*Fig. 3.*



INVENTOR.

EDWIN H. O'NEIL

BY

*Stockbridge & Co.*  
ATTORNEYS

## UNITED STATES PATENT OFFICE.

EDWIN H. O'NEIL, OF BROOKLYN, NEW YORK, ASSIGNOR, BY DIRECT AND MESNE ASSIGNMENTS, OF ONE-HALF TO CHARLES E. BILL, OF NEW YORK, N. Y.

## DEODORANT AND METHOD OF MAKING SAME.

Application filed November 27, 1923. Serial No. 677,223.

An object of my invention is to provide a deodorant which will be effective in stopping or destroying odors of perspiration, which will be hygienic, which may be applied with facility and convenience, which will be non-greasy and harmless to the clothing, and which will be easy and inexpensive to produce.

Many deodorants now on the market are in the form of salves, powders or liquids containing astringents which operate to close the pores and thus check the perspiration, some being scented or perfumed so that their own conspicuous odors render the odors of perspiration inappreciable. It is a fact well known that there is a certain danger attendant upon artificially closing the pores, and it is also recognized that the perfumed and scented odors frequently become objectionable, particularly when mingled with that of perspiration. There is an obvious disagreeable feature about applying salves, and because of the greasy nature of the salves and many of the liquids they will rub off on the clothing unless some protection is provided, which is not always possible to do. Powders are also disadvantageous for the reason that they do not have the quality of adhering and hence they are both wasteful and inconvenient of application.

By my invention I am able to make a deodorant in solid cake or stick form which can be applied to any portion of the body by merely rubbing it over the parts, such as under the armpits or between the toes. The nature of my product is such that it does not crumble but rubs off easily in a smooth even film, and yet is not greasy to any objectionable degree. Furthermore, while it is itself practically odorless, it has the property of destroying the characteristic odor of the perspiration. It does not have any astringent action upon the pores, it does not soil the fingers, does not rub off on the clothing, is invisible when applied and retains its solidity at any atmospheric temperature.

The deodorant constituents of my product are zinc oxide and boric acid, preferably in substantially equal amounts by weight. While the deodorant properties of these substances individually have been heretofore known, I believe that I am the first to have

recognized the superior results which are obtained by combining them in the proper proportions, and I furthermore believe that I am the first to have been able to produce a solid cake or stick containing these substances in such quantities as to be effective as a deodorant and which at the same time is non-greasy in its nature and yet can be applied in a thin film or layer without crumbling.

I have found that the best body or binder for the deodorant powders is spermaceti which is made slightly soft or pliable by a proper amount of a petroleum jelly. While other waxy substances might perhaps be employed as the binder to produce the solid form of the product, I have not been able to obtain entirely satisfactory results with other than spermaceti and petrolatum combined in about two parts by weight of the former to one part of the latter. The product is improved by adding a few drops of petroleum oil to the mixture.

My invention also contemplates a method of combining the powders with this binder so as to afford the maximum quantity of the powders and at the same time make a product in which the powders are evenly distributed and which will rub off smoothly without crumbling. I have found that when the product is properly made it can readily be molded to the desired shape of sticks or cakes, and a convenient shape of the product, which my invention includes, is a flat, oval stick having a round end. A stick of this shape has the advantage that when applied to the concavities of the body, as, for example, in the armpits, it conforms to the shape of that part of the body and may be applied thereto with one or two sweeps of the stick over the part.

In the drawings, I have shown one form in which the product may be molded in accordance with my invention, Figure 1 being an elevation of the stick; Figure 2 being a top end view; and Figure 3 being a bottom end view thereof.

In accordance with my invention I first melt a quantity of spermaceti having mixed therewith a sufficient quantity of petrolatum, such as vaseline, which gives the desired consistency to the product when it is hardened. As above stated, substantially two parts by weight of the spermaceti to one of

the vaseline gives the best results, and the product will be further improved by adding a few drops of petroleum oil, such as white mineral oil. The spermaceti should be melted slowly and the molten mixture should be raised to a temperature of from 140° to 150° F. I then take a powder containing an equal mixture by weight of zinc oxide and boric acid and stir into the molten liquid a quantity thereof substantially equal in weight to that of the molten liquid. This powder should be poured in slowly and the liquid should be constantly stirred as the powder is entering it. If the temperature of the molten liquid is properly regulated a homogeneous and stable mixture will thus be obtained. If the temperature is too low the liquid will not be sufficiently thin to permit of a thorough mixture of the powder therein, while if the temperature is substantially above 150° F. the result is a curdling action.

While the spermaceti will melt at about 110° F., the temperature of the molten liquid is lowered by the addition of the cold powder, and it is therefore necessary to have the initial temperature sufficiently high to leave the mass in a molten condition after the powder is stirred in. I have found that a quantity of the powder equal by weight to substantially 50% of the entire mass will reduce the temperature from around 145° to around 115° F. This is, therefore, substantially the maximum amount of powder that can be used for the reason that the liquid cannot safely be at a temperature substantially above 150° F. when the powder is stirred in.

After the powder is stirred into the molten liquid, the mass is poured into suitable molds, where it quickly hardens. In fact, the material hardens so quickly that it is desirable to provide a heat insulating jacket around the body while pouring the liquid into the molds. I have found that aluminum molds are entirely satisfactory. Bakelite molds are also satisfactory, although more expensive.

I prefer to make the molds of a shape to produce the stick illustrated in the drawings. The stick A of the solid deodorant material produced as above described, is of a flat, oval shape with a rounded end, the major axis of the oval being conveniently about one and one-quarter inches in length. While this at ordinary temperatures is entirely nongreasy and will not soil the fingers, it does yield to the temperature of the body and will rub off when pressed hard against the part. For this reason, in order to protect the fingers of the user, I prefer to cover the lower end of the stick with a suitable protective wrapping B. This makes a handy and compact form for the material.

While my invention is not limited to any

exact or very careful proportions, an excellent product is produced from the following formula by weight of the constituents: 25% zinc oxide, 25% boric acid, 33% spermaceti, 16 1/4% vaseline, 1/4 of 1% white petroleum oil.

Without the petroleum products, it is evident that the stick or cake will tend to crumble when rubbed over the skin, particularly when the stick is relatively cold. The vaseline and white petroleum oil in the proportions stated make the product just soft enough to rub off smoothly at any temperature without making the product greasy to the touch.

In order to make the product less visible when applied to the skin than would be if left in its natural white color, a small quantity of a pinkish coloring material, such as an oil soluble aniline dye, may be added thereto to cause the product to simulate a flesh color.

In addition to its property of stopping the odors of perspiration without clogging the pores, and of reducing excessive perspirations to normal, my improved deodorant is refreshing, soothing and healing, being a good antiseptic for minor cuts and sores.

It is evident that, if desired, the proportion between the zinc oxide and boric acid may be changed, and that other changes may be made and equivalents may be substituted for the constituents mentioned without departing from the spirit of my invention as expressed in the following claims.

I claim:

1. A deodorant to be applied to the body composed by weight of substantially one part each of zinc oxide and boric acid and two parts of a waxy binder containing substantially two parts of a wax and one of petrolatum, molded in stick form and adapted to rub off in a smooth even film when applied.

2. A deodorant in solid form composed by weight of substantially 25% zinc oxide, 25% boric acid, 33% spermaceti, 16 1/4% of petroleum, and 1/4 of 1% petroleum oil.

3. A deodorant to be applied to the body comprising by weight substantially 25% zinc oxide, 25% boric acid, 33% spermaceti, 16 1/4% petrolatum and 1/4 of 1% petroleum oil molded into solid stick form and adapted to rub off in a smooth even film when applied.

4. The process consisting in heating together substantially two parts by weight of spermaceti and one part of petrolatum until the mixture is in a molten condition at substantially 145° F., then stirring in a quantity of a mixture of zinc oxide and boric acid substantially equal in weight to the molten liquid, then cooling and molding the mixture into a solid stick form.

5. The process consisting in raising to

substantially 145° F. a waxy compound composed by weight of substantially two parts of spermaceti and one of petrolatum and less than one percent of petroleum oil, then slowly adding and stirring in a quantity of a powder substantially equal by weight to that of the molten liquid and composed of sub-

stantially equal parts of zinc oxide and boric acid, then cooling and molding the mixture into solid stick form.

In witness whereof, I hereunto subscribe my signature.

EDWIN H. O'NEIL.